

# United States Patent Office

2,753,263

Patented July 3, 1956

1

2,753,263

## SILVER HALIDE EMULSION CONTAINING A POLYMERIC POLYAMINE AS AN ACID DYE MORDANT

Russell Houston Gray, Middletown Township, Monmouth County, N. J., assignor to E. I. du Pont de Nemours and Company, Wilmington, Del., a corporation of Delaware

No Drawing. Application September 10, 1953,  
Serial No. 379,467

16 Claims. (Cl. 95—7)

This invention relates to photography and more particularly to photographic materials containing mordanting agents. Still more particularly, it relates to photographic elements having at least one water-permeable colloid silver halide emulsion containing a polymeric polyamine having at least one unsubstituted hydrogen atom on the amine group. The invention also relates to processes of mordanting and dye images utilizing such materials.

Various methods are known for mordanting acid dyes to water-permeable colloid layers in photographic elements. These methods utilize both inorganic and organic compounds. In case of organic compounds, many of them which are useful in textile mordanting procedures are not useful in photographic emulsions because the compounds have a deleterious effect on the silver halide grains. Polymeric quaternary salts have been proposed for the mordanting of acid dyes in the form of photographic images, but they have the disadvantage of causing excessive fog and affect the speed of the photographic emulsion. Polymeric quaternary salts also markedly affect the viscosity and consequently the coating characteristics of the molten emulsion. Consequently, they can only be safely used in nonsensitive layers of photographic elements.

An object of this invention is to provide improvements in the art of mordanting acid dyes in photographic silver halide emulsion layers. Another object is to provide new photographic film and paper elements wherein the silver halide emulsion layers contain polymeric nitrogenous compounds which do not have a deleterious effect on the silver halide grains. A further object is to provide such materials from readily available organic compounds. A still further object is to provide such materials which do not fog or lose their speed upon storage. Still other objects will be apparent from the following description of the invention.

It has been discovered that photographic films and papers having a strong mordanting action on acid dyes can be made by incorporating in the water-permeable silver halide emulsions thereof a polymeric polyamine having a main polymer chain consisting solely of carbon atoms and containing a plurality of amino groups in which the amino nitrogen has at least one hydrogen atom. The polymeric polyamines in question are selected from the class consisting of (a) polymeric polyamines in which the amino nitrogen, having at least one hydrogen atom, is directly attached by a single bond to a carbon atom of the main polymer chain, and (b) polymeric polyamines containing primary amino nitrogen atoms linked to a carbon atom of the main polymer chain through a methylene ( $—CH_2—$ ) group. Mixtures of two or more of the polyamines can be used.

The polymeric polyamines described in the foregoing paragraph are characterized by having a main polymer chain consisting solely of carbon atoms and further char-

2

acterized by having recurring substituent groups of the formula:



wherein  $\text{R}_1$  is H or an alkyl radical of 1 to 12 carbon atoms, i. e., methyl, ethyl, propyl, butyl, pentyl, hexyl, heptyl, octyl, nonyl, decyl, undecyl and dodecyl; and  $x$  is the cardinal number of 0 or 1. The compounds comprehended by this general formula have molecular weights from 300 to 50,000.

The polymeric polyamines used in accordance with one aspect of this invention are obtained by the reductive amination of a monoolefin/carbon monoxide polymer. These polymeric polyamines have a main polymer chain consisting solely of carbon atoms and contain as lateral substituents a plurality of amino



groups, where  $\text{R}_1$  has the same meaning as above, attached directly to a carbon atom of the main polymer chain. These compounds, when exemplified by those made by the reductive amination of ethylene/carbon monoxide polymers, have a plurality of units of the following general formula:



where  $n$  is an integer from 3 to 40 and  $\text{R}_1$  has the same significance as in Formula I. In the case of polymers made from other olefins, they will have similar structures except that the  $—\text{CH}_2—\text{CH}_2—$  is replaced by a



radical or a



radical where propylene and isobutylene are used as the olefin.

In another important aspect of the invention, the polymeric polyamines used in the silver halide dispersions are obtained by the reduction of a linear polymer containing units selected from the group consisting of acrylonitrile and alpha-methacrylonitrile units, said polymeric polyamine having a main polymer chain consisting solely of carbon atoms with the primary amino ( $—\text{NH}_2$ ) groups attached to the said main polymer chain through methylene ( $—\text{CH}_2—$ ) groups which are lateral substituents thereon. These compounds as exemplified by butadiene/acrylonitrile or alpha-methacrylonitrile copolymers are composed of a plurality of units having the Formulae III and IV below:



and

wherein  $n$  is a positive integer of 1 to 10.

The polymeric polyamines described above that are useful in accordance with the present invention may be made after the manner described in Hoehn U. S. 2,495,255 patented January 20, 1950, and Pinkney U. S. 2,585,583 patented February 12, 1952. The useful polymeric polyamines, however, may have a neutralization equivalent from 50 to 1,000 but preferably have a neutralization equivalent in the range from 150 to 500. By neutralization equivalent is meant the weight of polyamine required to neutralize one equivalent weight of any strong acid.

The photographic elements, e. g., film or paper bearing at least one water-permeable colloid silver halide emulsion containing one or more of the polymeric polyamines described above can be made in various manners. Thus the photographic films or paper can be made by any conventional method and the polymeric polyamine introduced into the photographic emulsion layer by impregnating it with an aqueous solution of the polymeric polyamine. Since the addition salts of the polymeric polyamines have a markedly higher solubility than the free bases, the polyamines are generally added in the form of the addition salt. This is conveniently done by dissolving the polymeric polyamine in aqueous acid, e. g., dilute aqueous acetic acid and impregnating the water-permeable colloid silver halide emulsion layer with the resulting solution.

Alternatively, the polymeric polyamines can be added to the water-permeable colloid silver halide emulsion prior to coating, that is, an emulsion which is made in the usual manner is admixed with an aqueous solution containing an addition salt, e. g., acetic acid salt of the polymeric amine.

The water-permeable colloids used in the emulsions may be any of the usual colloids used by photographic manufacturers. Thus the colloid may be gelatin, agar-agar, albumin, polyglycuronic acid, zein, collodion, polyvinyl alcohol, partially hydrolyzed polyvinyl acetate and interpolymers thereof with unsaturated materials such as ethylene, styrene, maleic acid, etc. which have hydrophilic properties, polyvinyl acetals, e. g., the acetal of polyvinyl alcohol with acetaldehyde or benzaldehyde or water-soluble or hydrophilic cellulose derivatives. Suitable hydrophilic or water-permeable colloids of the above types are described in U. S. Patents 2,110,491, 2,211,323, 2,276,322, 2,276,323, 2,286,215 and 2,397,866.

The proportion of polymeric polyamine to water-permeable colloid silver halide emulsion may vary over a fairly wide range. Thus from 2.0 to 100.0 grams of the mordant (the polymeric polyamine) in the form of the acid addition salt may be used for each 100 grams of gelatin or other water-permeable colloid used as the binding agent in the emulsion.

The invention will be further illustrated but is not intended to be limited by the following examples:

#### Example I

A gelatino silver chloride emulsion of a kind suitable for preparing a photographic printing paper of the contact type was made and 3 one-liter portions were separated. To these 3 emulsions there were added, from a 2% aqueous acetic acid solution, 1.25, 2.5 and 5.0 grams of the acetic acid addition salt of the polyamines obtained by the reductive amination of the polyketones prepared by the copolymerization of ethylene and carbon monoxide in the ratios of 6 to 1, 6.9 to 1 and 10.4 to 1,

respectively. These polyamines had molecular weights of 660, 1100 and 1480 and neutralization equivalents of 574, 352 and 506, respectively. They were prepared after the manner described in Hoehn U. S. Patent No.

5 2,495,255. The three aqueous emulsions were coated onto a baryta-coated sheet of paper and dried. The resulting photographic papers were exposed to light and then fixed in a 24% aqueous solution of  $\text{Na}_2\text{S}_2\text{O}_3 \cdot 5\text{H}_2\text{O}$ , washed and dried. The three papers were then treated

10 in an acid dye solution of the following composition:

|                                                    | Grams |
|----------------------------------------------------|-------|
| Pontacyl Carmine 6B (Colour Index 57)              | 1.2   |
| $\text{NaH}_2\text{PO}_4 \cdot \text{H}_2\text{O}$ | 15.0  |
| $\text{H}_2\text{O}$ to make 1.0 liter.            |       |

15 and washed for 15 minutes. It was found that each of the photographic papers were fastly dyed by the acid magenta dye. The photographic emulsion containing the polymeric amine having the neutralization equivalent of 352 retained the greatest amount and that having the neutralization equivalent of 574 the least amount of dye.

#### Example II

An aqueous gelatino silver chloride emulsion of the kind used in making photographic printing papers of the contact type was prepared and divided into several portions. A polymeric polyamine obtained by the reduction of a butadiene/acrylonitrile copolymer of 4 to 1 mol ratio and having a neutralization equivalent of 378 was dissolved in 2% aqueous acetic acid to form the acetic acid addition salt. No added ingredients were made to one control portion of the emulsion and chrome alum was added to a second portion. This solution was added in the quantities given in the following table to further respective portions of the silver chloride emulsion. These portions were then coated onto a baryta-coated sheet of paper. The respective photographic papers were exposed to a standard negative and then developed for one minute in a solution made of the following constituents:

|                                  | Grams |
|----------------------------------|-------|
| N-methyl-p-aminophenol sulfate   | 1.0   |
| Sodium sulfite                   | 15.0  |
| Hydroquinone                     | 4.0   |
| 45 Sodium carbonate (desiccated) | 22.5  |
| Potassium bromide                | 0.63  |
| Water to make 1.0 liter.         |       |

50 with the results given in the following table:

|    | Grams Polyamine Acetate Salt Per Liter of Emulsion | Print Speed (Seconds of Exposure) |                  |
|----|----------------------------------------------------|-----------------------------------|------------------|
|    |                                                    | 3.5 Months Aging at—              |                  |
|    |                                                    | Fresh                             | Room Temperature |
| 55 |                                                    |                                   |                  |
| 60 | None                                               | 20                                | 25               |
|    | 1.42                                               | 19                                | 20               |
|    | 2.84                                               | 17                                | 18               |
|    | 5.68                                               | 19                                | 20               |
|    | 1.42 gm. chrome alum                               | 25                                | 35               |

65 The data given in the above table show that the polyamines stabilize the emulsion to speed loss upon aging. No deleterious fog effects were noted either fresh or after aging.

70 Samples of the photographic papers just described were fixed in a 24% aqueous solution of  $\text{Na}_2\text{S}_2\text{O}_3 \cdot 5\text{H}_2\text{O}$ , washed and then dyed for 60 seconds in an aqueous solution containing a magenta acid dye of the type described in Example I. The dyed samples were cut in half, one half was rinsed in water and dried and the dye densities ( $d_1$ ) determined and the other half washed vigorously in water for a period of 30 minutes and dried

and the dye densities ( $d_2$ ) determined, with the results given in the following table:

| Mordant        | Grams Poly-amine Acetate Salt Per Liter of Emulsion | Percent Decrease in Dye Density ( $\frac{d_1 - d_2}{d_1} \times 100$ ) |
|----------------|-----------------------------------------------------|------------------------------------------------------------------------|
| None           | 0                                                   | 80.0                                                                   |
| Polyamine salt | 1.42                                                | 65.3                                                                   |
| Do.            | 2.84                                                | 18.7                                                                   |
| Do.            | 5.65                                                | 0                                                                      |
| Chrome alum    | 1.42                                                | 72.0                                                                   |

It should be noted that while chrome alum is an effective mordant, it has the disadvantage that it causes rapid hardening of the emulsion so that often coating cannot be accomplished due to such hardening.

### Example III

A gelatino silver iodobromide emulsion of the positive type was prepared for coating. It was divided into portions. To respective portions there were added 3.66 grams of the polyamines listed below per 100 grams of gelatin. The resulting emulsions were coated onto a cellulose triacetate film base bearing a thin gelatin anchor layer and dried. The resulting film elements were fixed in 24% aqueous  $\text{Na}_2\text{S}_2\text{O}_3 \cdot 5\text{H}_2\text{O}$  solution, washed, dried and dipped into a magenta dye solution of the type given in Example I for a period of ten minutes. The films were cut in half and one half was quickly rinsed in water and the other half washed for a period of one hour. The two halves were dried and the dye densities determined as in Example II with the results given in the following table:

| Polymeric Polyamine Mordant | Neutralization Equivalent | Percent Decrease in Dye Density, 1-Hour Washing |
|-----------------------------|---------------------------|-------------------------------------------------|
| a                           | 316                       | 81                                              |
| b                           | 365                       | 79                                              |
| c                           | 433                       | 87                                              |
| d                           | 506                       | 91                                              |

(a) This polymeric polyamine was obtained by the reduction of a butadiene/acrylonitrile copolymer of 4 to 1 mol ratio and was used in the form of the acetic acid addition salt which was made by dissolving the polyamine in 3% aqueous acetic acid.

(b) This polymeric polyamine was obtained by the reduction of a butadiene/methacrylonitrile copolymer of 4 to 1 mol ratio and was used in the form of the acetic acid addition salt which was made by dissolving the polyamine in 3% aqueous acetic acid.

(c) This polymeric polyamine is the same type as (b) but has a 4.5 to 1 mol ratio.

(d) This polymeric polyamine is the same as that described in Example I being made from the reductive amination of the ethylene/carbon monoxide polymerization product.

Each of the polymeric polyamines, a, b and c were made after the manner described in U. S. Patent No. 2,585,583. The polymeric amide (d) was made after the manner described in U. S. Patent No. 2,495,255.

Photographic films of the type described in Example III are useful in making cine color prints by imbibition dye transfer procedures. Thus, a dry matrix film can be introduced into a dye bath containing any suitable acid dye of the appropriate color and dyed. The dyed matrix is rinsed in water or dilute acetic acid and the excess blown off. A premordanted film of the type described in Example III is soaked in water at pH 7 for 10 seconds at 70° F. The dyed matrix is then contacted with the premordanted film. The matrix and mordanted films are left in emulsion contact for a period of about one minute at 100 to 150° F. The two films are then stripped apart and the matrix washed in water and either dried for storage or redyed for a further imbibition printing process.

### Example IV

A gelatino silver iodobromide emulsion of the positive type was prepared for coating. It was divided into two

equal portions. No mordant was added to one portion and to the other portion there was added 14.8 grams of the polymeric amine of butadiene/methacrylonitrile having a neutralization equivalent of 365 described under (b) of Example III per 100 grams of gelatin. The resulting emulsions were coated onto cellulose triacetate bases bearing a thin anchoring layer and dried. The resulting light-sensitive elements were exposed and processed as follows:

10 The element was developed for 3½ minutes in a developer of the following composition:

| Grams                                              |
|----------------------------------------------------|
| N-methyl-p-aminophenol sulfate                     |
| Na <sub>2</sub> SO <sub>3</sub>                    |
| 15 Hydroquinone                                    |
| Na <sub>2</sub> CO <sub>3</sub> · H <sub>2</sub> O |
| KBr                                                |
| Water to make 1.0 liter.                           |

20 The element was then rinsed and fixed in a solution having the following composition:

| Grams                                                                                 |
|---------------------------------------------------------------------------------------|
| Sodium thiosulfate, Na <sub>2</sub> S <sub>2</sub> O <sub>3</sub> · 5H <sub>2</sub> O |
| Sodium sulfite                                                                        |
| 25 Sodium bisulfite                                                                   |
| Water to make 1.0 liter.                                                              |

25 The element was washed and dried. A matrix film bearing a relief image of a resolution chart was dyed in an acid dye bath. It was then rinsed in a 1% acetic acid solution and brought into intimate contact with a sample of the premordanted film which had been previously soaked for 10 seconds in water. The two films were held in intimate contact for 30 seconds at 150° F. and then separated. They were rinsed in 1% acetic acid and dried. The other sample processed above was treated in the same way. The resolution in terms of lines per millimeter of the resultant transferred dye image which is a measure of mordanting power was determined microscopically and found to be as shown in the following table:

| Mordant (grams/100 grams of gelatin) | Resolution (lines/millimeter) |
|--------------------------------------|-------------------------------|
| none                                 | 11                            |
| 14.8                                 | 25                            |

### Example V

30 An emulsion prepared as in Example III was divided into three parts and 27 grams per hundred grams of gelatin of each of the acetate, and iodide salts of the polymeric amine of butadiene/methacrylonitrile copolymer (BD/MAN) described under (b) of Example III were added to two of the divided parts respectively. The fifth portion contained no mordanting agent. The samples were processed and tested as shown in Example IV except that the samples were also submitted to one hour washing as in Example III and the following results were observed.

| Mordant         | Percent dye lost in 1 hour washing | Resolution (lines/millimeter) |
|-----------------|------------------------------------|-------------------------------|
| BD/MAN acetate  | 32                                 | 25.                           |
| BD/MAN bromide  | 17                                 | not determined.               |
| BD/MAN chloride | 27                                 | Do.                           |
| BD/MAN iodide   | 15                                 | 33.                           |
| no mordant      | 99                                 | 11.                           |

70 In place of the specific polymeric polyamines given in the foregoing examples one may substitute other polymeric amines described in the foregoing patents having the requisite neutralization equivalent. Additional useful polyamines include isobutylene/ethylene/carbon monoxide polymeric amine, propylene/ethylene/carbon monox-

7  
ide polymeric amine, isobutylene/carbon monoxide polymeric amine, propylene/carbon monoxide polymeric amine, and polyallylamine.

The mordanted films and papers of this invention are useful in various types of dye printing or imbibition printing operations. Thus, they are useful in the preparation of three color dye transfer prints on paper supports, in the preparation of monochrome dyed prints for special effects and for hand colored color prints.

The present invention is not limited to the use of a barya-coated paper or a cellulose triacetate film base as the water-permeable silver halide layers containing the polymeric polyamines can be deposited on various supports. Thus, the support may be composed of practically any type of transparent film or any type of paper which is resistant to photographic processing solutions. Thus, the film may be composed of superpolymers, e. g., linear polyamides, cellulose nitrate, polyvinyl acetals, cellulose propionate, cellulose mixed esters, cellulose ethers, vinyl chloride and copolymers, styrene, acrylonitrile and copolymers, polyesters, e. g., polyethylene terephthalates, vinyl acetate and copolymers, vinyl fluoride and copolymers, polyvinyl alcohol; transparentized paper, etc. The coated film base of Alles et al. 2,627,088 is especially useful.

The photographic films and papers of this invention have the advantage that they have a strong mordanting action on acid dyes. A further advantage resides in the fact that the polymeric polyamines cause little or no fog in the resulting light-sensitive silver halide emulsion layers. A still further advantage resides in the fact that the polymeric polyamines do not adversely affect the stability of the resulting emulsions. Thus, no significant loss of speed or fogging occurs upon aging of the film elements. Another advantage of the invention is that the mordants are easy to use and do not have a significant hardening action on the conventional types of water-permeable colloids. A further advantage lies in the fact that polyamines have little or no effect on the physical characteristics of molten photographic emulsions before coating.

What is claimed is:

1. A photographic element comprising a support bearing at least one water-permeable colloid silver halide emulsion layer containing at least one polymeric polyamine containing carbon, hydrogen and nitrogen atoms only and having a main polymer chain consisting solely of carbon atoms, said polyamines being taken from the class consisting of polymeric polyamines in which the amino nitrogen atom has at least one hydrogen atom attached thereto and is directly attached by a single bond to a carbon atom of the main polymer chain and polymeric polyamines containing amino nitrogen atoms directly attached to a carbon atom of the main polymer chain through a single methylene group, said amino nitrogen atoms having at least one hydrogen atom attached thereto, said polyamine having a molecular weight from 300 to 50,000 and a neutralization equivalent from 50 to 1,000.

2. A photographic element comprising a flexible sheet bearing at least one water-permeable colloid silver halide emulsion layer containing a polymeric polyamine having a polymer chain consisting solely of carbon atoms in which the amino nitrogen atom has at least one hydrogen atom attached thereto and the nitrogen atom is directly attached by a single bond to the carbon atom of the main polymer chain, said polyamine having a molecular weight from 300 to 50,000 and a neutralization equivalent from 50 to 1,000.

3. An element as set forth in claim 2 wherein said sheet is a barya-coated paper.

4. An element as set forth in claim 2 wherein said sheet is a hydrophobic film base.

5. A photographic element comprising a flexible sheet bearing at least one water-permeable colloid silver halide emulsion layer containing a polymeric polyamine consisting of carbon, hydrogen and nitrogen atoms only and

5  
having a polymer chain consisting solely of carbon atoms containing primary amino nitrogen atoms directly attached to a carbon atom of the main polymer chain through a single methylene group, said polyamine having a molecular weight from 300 to 50,000 and a neutralization equivalent from 50 to 1,000.

6. An element as set forth in claim 5 wherein said sheet is a barya-coated paper.

7. An element as set forth in claim 5 wherein said sheet is a hydrophobic film base.

8. A photographic element comprising a flexible sheet bearing a water-permeable colloid silver halide emulsion layer containing a polymeric polyamine having a polymer chain consisting solely of carbon atoms having, as the sole units in the polymer chain, recurring intralinear units of the formula:



25  
wherein  $n$  is a positive integer of 3 to 40 and  $\text{R}_1$  is a member taken from the group consisting of hydrogen and alkyl of 1 to 12 carbon atoms, said polyamines having a molecular weight from 300 to 50,000 and a neutralization equivalent from 150 to 500.

30  
9. A photographic element comprising a flexible sheet bearing a water-permeable colloid silver halide emulsion layer containing a polymeric polyamine having a polymer chain consisting solely of carbon atoms having, as the sole units in the polymer chain, recurring intralinear units of the formula:



40  
wherein  $n$  is a positive integer of 1 to 10, said polyamines having a molecular weight from 300 to 50,000 and a neutralization equivalent from 150 to 500.

45  
10. A photographic element comprising a flexible sheet bearing a water-permeable colloid silver halide emulsion layer containing a polymeric polyamine having a polymer chain consisting solely of carbon atoms having, as the sole units in the polymer chain, recurring intralinear units of the formula:



55  
wherein  $n$  is an integer of 1 to 10 said polyamines having a molecular weight from 300 to 50,000 and a neutralization equivalent from 150 to 500.

60  
11. A photographic film comprising a flexible hydrophobic film base bearing at least one gelatin silver halide emulsion layer containing a polymeric polyamine having a polymer chain consisting solely of carbon atoms having, as the sole units in the polymer chains, recurring intralinear units of the formula:



70  
wherein  $n$  is an integer of 3 to 40, said polyamines having a molecular weight from 300 to 50,000 and a neutralization equivalent from 150 to 500.

75  
12. A film element as set forth in claim 11 wherein said base is composed of a polyethylene terephthalate.

13. A photographic film comprising a flexible hydrophobic film base bearing at least one gelatin silver halide emulsion layer containing a polymeric polyamine having a polymer chain consisting solely of carbon atoms having,

as the sole units in the polymer chain, recurring intra-linear units of the formula:



5

wherein  $n$  is a positive integer of 1 to 10, said polyamines having a molecular weight from 300 to 50,000 and a neutralization equivalent from 150 to 500.

14. A film element as set forth in claim 12 wherein said film base is composed of polyethylene terephthalate.

15. A photographic film comprising a flexible hydrophobic film base bearing at least one gelatin silver halide emulsion layer containing a polymeric polyamine having a polymer chain consisting solely of carbon atoms having, as the sole units in the polymer chain, recurring intra-linear units of the formula:



20

wherein  $n$  is a positive integer of 1 to 10, said polyamines having a molecular weight from 300 to 50,000 and a neutralization equivalent from 150 to 500.

16. A photographic film as set forth in claim 15 wherein said film base is composed of polyethylene terephthalate.

**References Cited in the file of this patent**

**UNITED STATES PATENTS**

2,423,460 McQueen \_\_\_\_\_ July 8, 1947  
2,486,191 Minsk et al. \_\_\_\_\_ Oct. 25, 1949

**FOREIGN PATENTS**

648,472 Great Britain \_\_\_\_\_ Jan. 3, 1951